

## UNITED STATES PATENT OFFICE

2,453,087

PHOTOGRAPHIC DEVELOPERS CONTAINING  
TETRAZOLYL DISULFIDES AS ANTIFOG-  
GING AGENTSFritz Dersch and Robert H. Clark, Binghamton,  
N. Y., assignors to General Aniline & Film Cor-  
poration, New York, N. Y., a corporation of  
DelawareNo Drawing. Application November 7, 1946,  
Serial No. 708,474

16 Claims. (Cl. 95—88)

1

This invention relates to photographic developers containing anti-fogging agents, and more particularly to the use of tetrazolyl disulfides as such agents in developers.

It is known in the art that light-sensitive emulsions, such as gelatin silver-halide emulsions, have a decided tendency to fog. The fog may be of two types, namely, yellow fog and chemical (gray) fog. The yellow fog, sometimes referred to as color fog or dichroic fog, is essentially a colloidal deposit of silver, the color intensity and general appearance of which are determined by the minute particle size and degree of subdivision. The fog is chiefly yellow in color and is most apparent in the lighter portions of a negative. The color may vary, however, and the colloidal silver particles may, for example, appear green by reflected light and yellow or red by transmitted light. The so-called chemical fog, or gray fog, on the other hand, is the more common and is formed in a number of ways. It may be caused by premature exposure, by excessive ripening of the emulsions, or by the storage of the film, particularly at high temperatures or for unusually long periods of time.

When photographic plates and films coated with gelatin silver-halide emulsions are allowed to age for periods of time prior to processing, a chemical fog thereafter appears in the unexposed areas upon development. This fog occurs to a somewhat lesser extent when the plate or film is exposed and developed immediately after coating, providing the plate or film is given a normal period of development. It occurs to a much greater extent if the period of development be unusually long.

It is also known that mercapto tetrazoles and tetrazoles containing at least one  $=\text{NH}$  group, the hydrogen atom of which is capable of substitution by silver, are effective in preventing an increase in fog and are thus effective in stabilizing or controlling the keeping quality of light-sensitive silver-halide emulsions. Although these compounds have the ability to give the emulsions to which they are added stability and a steeper gradation, they have a definite shortcoming in that they, to some extent, lower the sensitivity of the emulsions.

The primary object of the present invention is to provide stabilizers or fog inhibiting agents which are incorporated in the developing bath or in a separate processing bath.

A further object is to provide stabilizers or fog inhibiting agents which are incorporated into a black and white or color developer and which tend

2

to prevent the formation of chemical fog in light-sensitive silver-halide emulsions without lowering the sensitivity of such emulsions.

A still further object is to reduce the amount of chemical fog produced upon development of a silver-halide emulsion by developing said emulsion with a developer containing a fog-inhibiting amount of tetrazolyl disulfide.

Other objects and advantages will appear from the following specification.

We have found that by combining in a single compound, both the tetrazole and disulfide radical in the form of a tetrazolyl disulfide, components are obtained which are far superior in fog reducing action to either radical when used in conjunction with some other group. Such compounds may be termed bis(1-substituted-tetrazolyl-5-) disulfides and have the following structural formula:



where  $R$  is a hydrocarbon radical, e. g., methyl, ethyl, propyl, isopropyl, butyl, isobutyl, sec.-butyl, tert.-butyl, amyl, hexyl, heptyl, octyl, nonyl, allyl, propargyl, butenyl, pentenyl, hexenyl, phenyl, o-, m-, and p-tolyl, naphthyl,  $\alpha$ -naphthyl,  $\beta$ -naphthyl, diphenyl, benzyl, methyl benzyl, ethyl benzyl, and the like.

There are two general methods by which the tetrazolyl disulfides may be prepared. The first method applies to those tetrazolyls where  $R$  in the above general formula is aliphatic, and the second method to those where  $R$  is aromatic.

The first method is described by R. Stollé in the Journ. für prakt. Chemie, 133, p. 60, 1932, and consists of adding dropwise a solution of any aliphatic isothiocyanate in 95% alcohol to a hot, well-stirred, alcoholic suspension of sodium azide and heating the mixture under reflux for a period of time ranging from 2 to 8 hours. The reaction involved proceeds as follows:



wherein  $R$  and  $R_1$  are of the same value as  $R$  above.

During the reflux period, a strong stream of  $\text{CO}_2$  is passed through the well-stirred reaction mixture. At the end of the reflux period, the

mixture is filtered hot and the hot filtrate evaporated to dryness. The residue is taken up in water (filtered, if necessary) and extracted several times with ether. The water solution is freed of ether and then acidified with HCl. The acidified solution is evaporated to dryness and the solid or sticky residue is purified by crystallization from ether or chloroform to yield the mercaptan.



Oxidation of the mercaptan to the tetrazolyl disulfide proceeds thus:



and may be effected by treatment of the water solution of the mercaptan with ferric chloride solution or with hydrogen peroxide. The disulfide precipitates from solution and may be crystallized from alcohol.

The second method is described by the same author on page 61 of the same publication and is similar to the first method with the exception that any aromatic isothiocyanate is substituted for an aliphatic isothiocyanate, the passage of CO<sub>2</sub> is omitted, and the reflux time reduced to 2 hours. On acidification, a solid product precipitates. This is recrystallized directly to yield the mercaptan in pure form.

Oxidation of this mercaptan to the disulfide may be effected by treatment with hydrogen peroxide or dilute nitric acid. The resulting disulfide is best recrystallized from ethyl alcohol.

In the preparation of the tetrazolyl disulfides, utilized in accordance with the present invention, any aliphatic or aromatic isothiocyanate may be employed as the starting material. The nature of the isothiocyanate is immaterial, so long as the hydrocarbon radical is of the alkane, cycloalkane, alkene, alkynyl, or aryl type.

As examples of suitable isothiocyanates may be mentioned isothiocyanic acid methyl ester, ethyl ester, propyl ester, isopropyl ester, butyl ester, isobutyl ester, sec.-butyl ester, tert.-butyl ester, amyl ester, isoamyl ester, hexyl ester, heptyl ester, octyl ester, nonyl ester, decyl ester, allyl ester, propargyl ester, phenyl ester, benzyl ester, xenyl ester, o-tolyl ester, p-tolyl ester, and the like.

The following examples will serve to illustrate certain ways in which the stabilizers of our invention have been prepared and applied, but are not to be construed as limiting the invention.

#### Example I



Bis(1-methyltetrazolyl-5-)disulfide

An alcoholic solution of 15 grams of methyl isothiocyanate was added dropwise to a suspension of 19.5 grams of sodium azide in 250 cc. of 95% ethyl alcohol contained in a 3-necked, 1 liter, round-bottom flask fitted with an efficient stirrer, reflux condenser and inlet tube for the admission of CO<sub>2</sub>. The mixture was stirred well throughout this operation and the subsequent 8 hour reflux period. Carbon dioxide was then passed through

the mixture in a strong stream and the temperature of the mixture raised to the reflux point. Reflux was continued for 8 hours.

At the end of this time, the suspension was filtered while still hot and the alcoholic filtrate evaporated to dryness on a water bath under reduced pressure. The residue was taken up in water and extracted twice with 50 cc. portions of ether to remove unreacted methyl isothiocyanate.

10 The ether was removed from the aqueous solution by passing through it a stream of air. The aqueous solution was made acid (Congo red paper) with dilute hydrochloric acid, and the resulting solution evaporated to dryness on a water bath under reduced pressure. Extraction of the resulting mass with boiling chloroform, followed by chilling of the extract, resulted in the formation of white crystals of 1-methyl-5-mercaptotetra-

15 zole.

20 A solution of 2 grams of 1-methyl-5-mercaptotetrazole in 30 cc. of water was warmed for 10 minutes with a mixture of 2 cc. of 30% hydrogen peroxide and 5 cc. of water. On cooling the mixture in ice, a precipitate appeared which was filtered and crystallized from ethyl alcohol.

#### Example II



Bis(1-phenyltetrazolyl-5-)disulfide

A solution of 13.5 grams of phenyl isothiocyanate in 150 cc. of 95% ethyl alcohol was added dropwise to a well-stirred suspension of 10 grams of sodium azide in 50 cc. of absolute alcohol contained in a 3-necked, 500 cc., round-bottom flask equipped with an efficient stirrer and reflux condenser. The temperature of the well-stirred mixture was then raised to the reflux point and maintained there for two hours. At the end of this time, the mixture was filtered hot and the filtrate evaporated to dryness on the water bath under reduced pressure. The solid residue was taken up in water and the unreacted phenyl isothiocyanate removed by extraction with two 50 cc. portions of ether. The aqueous layer was acidified with dilute hydrochloric acid and the precipitate formed was collected on a Buchner funnel, washed with a little water and finally recrystallized from dilute ethyl alcohol.

55 Ten grams of the mercaptan was suspended in 500 cc. of a 10% nitric acid solution and, with good agitation, the temperature of the mixture raised to the boiling point. Immediately the suspension was filtered, the yellow solid remaining on the Buchner funnel was washed free of acid with water and crystallized from 95% ethyl alcohol.

#### Example III



Bis(1-allyltetrazolyl-5-)disulfide

Example I was repeated with the exception that 20 grams of allyl isothiocyanate was substituted for 15 grams of methyl isothiocyanate.

The tetrazolyl disulfides, which are substituted 75 in the 1-position by an aliphatic hydrocarbon

radical, are dissolved in alcohol, such as methyl, ethyl, propyl, and the like, or in a water mixture thereof, and the solutions thus obtained mixed with any black and white or color developer of the type used in the art in processing black and white and color film.

Where, however, the 1-position of the tetrazolyl disulfide is substituted by an aryl radical, such compound is best dissolved in a small quantity of acetone or dioxane, and the solutions thus obtained mixed with any one of the common black and white and color developers. The concentration of the fog inhibiting agent employed in either black and white or color developers may vary from about  $\frac{1}{2}$  to 500 mgs. per liter of developer or higher.

In order that those skilled in the art may better understand the nature and scope of this invention, the following specific examples are given without any intention of limiting the invention thereto.

#### Example IV

To one liter of a common developer solution, such as any standard p-monomethylamino-phenol-sulfate-hydroquinone formula, is added 30 mgs. of bis(1-methyltetrazolyl-5-) disulfide in 10 cc. of ethanol. A film having an emulsion which normally exhibits a tendency to form fog was developed in this solution without the formation of such fog.

#### Example V

A color developer for forming colored images by coupler development was made up as follows:

##### A

|                                     |       |      |
|-------------------------------------|-------|------|
| p-Aminodiethylaniline hydrochloride | grams | 2.5  |
| Sodium sulfite (anhydrous)          | do    | 1.0  |
| Sodium carbonate (monohydrate)      | do    | 67.5 |
| Potassium bromide                   | do    | 2.0  |
| Water to make                       | liter | 1    |

##### B

|                                      |       |      |
|--------------------------------------|-------|------|
| Bis(1-phenyltetrazolyl-5-) disulfide | grams | 0.2  |
| Acetone                              | cc.   | 20.0 |

For use solution B was added to solution A with rapid stirring.

A subtractive color positive film containing coupling agents in the emulsion layers, such as prepared according to United States Patents 2,179,228, 2,186,849, and 2,220,187, was exposed and developed in the color developer as above described.

It is to be noted that in cases where the emulsion layers do not contain coupling agents, the coupling agents are added to the color developer containing the fog inhibitor and the exposed silver-halide layers processed in the usual manner.

#### Example VI

Example IV was repeated with the exception that an equivalent quantity of bis(1-allyltetrazolyl-5-) disulfide was substituted for bis(1-methyltetrazolyl-5-) disulfide.

Special advantages are gained when films or plates, which have been stored at high temperatures or for unusually long periods of time, are developed in a developer, or washed or fixed in a bath containing our fog inhibitors.

Various modifications of this invention will occur to persons skilled in the art and it is, therefore, understood that the patent granted shall only be limited by the following claims.

We claim:

1. A photographic developer containing a developing agent and a fog inhibiting amount of a tetrazolyl disulfide having the general formula:



where R represents a hydrocarbon radical.

2. A photographic developer containing a developing agent and a fog inhibiting amount of a tetrazolyl disulfide having the formula:



20 3. A photographic developer containing a developing agent and a fog inhibiting amount of a tetrazolyl disulfide having the formula:



25 4. A photographic developer containing a developing agent and a fog inhibiting amount of a tetrazolyl disulfide having the formula:



30 40 5. A color-forming photographic developer comprising a primary aromatic amino developing agent and a fog inhibiting amount of a tetrazolyl disulfide having the general formula:



50 where R represents a hydrocarbon radical.

6. A color-forming photographic developer comprising a primary aromatic amino developing agent and a fog inhibiting amount of a tetrazolyl disulfide having the formula:



55 60 7. A color-forming photographic developer comprising a primary aromatic amino developing agent and a fog inhibiting amount of a tetrazolyl disulfide having the formula:



75 8. A color-forming photographic developer comprising a primary aromatic amino developing

agent and a fog inhibiting amount of a tetrazolyl disulfide having the formula:



9. The method of preventing the formation of fog upon development of an exposed silver-halide emulsion which comprises developing said emulsion with a developing agent containing, in a fog inhibiting amount, a tetrazolyl disulfide having the general formula:



where R represents a hydrocarbon radical.

10. The method of preventing the formation of fog upon development of an exposed silver-halide emulsion which comprises developing said emulsion with a developing agent containing, in a fog inhibiting amount, a tetrazolyl disulfide having the formula:



11. The method of preventing the formation of fog upon development of an exposed silver-halide emulsion which comprises developing said emulsion with a developing agent containing, in a fog inhibiting amount, a tetrazolyl disulfide having the formula:



12. The method of preventing the formation of fog upon development of an exposed silver-halide emulsion which comprises developing said emulsion with a developing agent containing, in a fog inhibiting amount, a tetrazolyl disulfide having the formula:



13. The method of preventing the formation of fog upon color development of an exposed silver-halide emulsion containing color-formers which comprises developing said emulsion with a developer containing a primary aromatic amino developing agent and, in a fog inhibiting amount, a tetrazolyl disulfide having the general formula:



where R represents a hydrocarbon radical, in the presence of a coupler compound.

14. The method of preventing the formation of fog upon color development of an exposed silver-halide emulsion containing color-formers which comprises developing said emulsion with a developer containing a primary aromatic amino developing agent and, in a fog inhibiting amount, a tetrazolyl disulfide having the formula:



in the presence of a coupler compound.

15. The method of preventing the formation of fog upon color development of an exposed silver-halide emulsion containing color-formers which comprises developing said emulsion with a developer containing a primary aromatic amino developing agent and, in a fog inhibiting amount, a tetrazolyl disulfide having the formula:



in the presence of a coupler compound.

16. The method of preventing the formation of fog upon color development of an exposed silver-halide emulsion containing color-formers which comprises developing said emulsion with a developer containing a primary aromatic amino developing agent and, in a fog inhibiting amount, a tetrazolyl disulfide having the formula:



in the presence of a coupler compound.

FRITZ DERSCH.  
ROBERT H. CLARK.

#### REFERENCES CITED

The following references are of record in the file of this patent:

#### UNITED STATES PATENTS

| Number    | Name    | Date           |
|-----------|---------|----------------|
| 1,962,123 | Brooker | June 12, 1934  |
| 2,124,159 | Weyde   | July 19, 1938  |
| 2,340,763 | McQueen | Feb. 1, 1944   |
| 2,385,762 | Mueller | Sept. 25, 1945 |
| 2,403,927 | Kendall | July 16, 1946  |